

## 1

3,126,342

### LUBRICATION OF THE MOVING PARTS OF INTERNAL COMBUSTION ENGINES OPERATING ON SULFUR AND OXYGEN OR OXYGEN-CONTAINING GASES

Gerhard Schachenmaier and Klaus Starke, Ludwigshafen (Rhine), Germany, assignors to Badische Anilin- & Soda-Fabrik Aktiengesellschaft, Ludwigshafen (Rhine), Germany

No Drawing. Filed Feb. 2, 1961, Ser. No. 86,573

Claims priority, application Germany Feb. 5, 1960

3 Claims. (Cl. 252—31)

The present invention relates to a method of lubricating the moving parts of internal combustion engines operating on sulfur and oxygen or oxygen-containing gases.

It is known to react sulfur with oxygen or oxygen-containing gases to sulfur dioxide in the combustion chamber of internal combustion engines and to directly convert the combustion heat evolved into mechanical energy.

If the moving parts of such internal combustion engines, where metal slides on metal, are lubricated with conventional lubricants, considerable trouble is caused, even after only short operating periods, by the small proportion of sulfur trioxide contained in the combustion gases. The sulfur trioxide attacks the lubricating oil with formation of organic sulfonic and sulfenic acids as well as the iron parts of the engine, as for example the piston rings and the working surface of the cylinder, with formation of viscous, tar-containing and strongly acid-reacting products which contain iron in the form of cations and some of which are water-soluble. These viscous, greasy substances gum up the piston rings so that they can no longer perform their sealing function. This causes strong blow-by into the crankcase and, as a result, the efficiency of the internal combustion engine is decreased considerably. The injurious effects produced by the sulfur trioxide contained in the combustion gases are aggravated by the action of sulfuric acid formed by the reaction of sulfur trioxide with water vapor which is contained in small amounts in the combustion gases and results from the combustion of lubricant.

We have found that the said disadvantages can be overcome by adding 0.05 to 10% by weight of elementary sulfur to the lubricant used in the internal combustion engine and maintaining the inner cylinder wall of the internal combustion engine at a temperature above the dew point of sulfuric acid. The upper limit to the temperatures that may be employed depends on the material of the cylinder wall and on the lubricant used. Within the said limits, the temperatures may be varied at will. Depending on the temperature range as well as on the lubricant used, the sulfur added is present in the lubricant in dissolved form or in the form of a suspension or emulsion.

## 2

The portion of sulfur trioxide which comes into contact with the lubricant is reduced to sulfur dioxide by the elementary sulfur that has been added to the lubricant and is thus rendered innocuous.

5 In order to ensure that the temperature of the cylinder wall does not fall below the dew point of sulfuric acid, the temperature of the cooling medium used for indirect withdrawal of the heat of combustion is maintained at 120° to 165° C., preferably at 145° to 155° C. If water at atmospheric pressure is used as the coolant, agents for elevating the boiling point, such as glycol, glycerol and the like, must be added to the cooling water in order to achieve the said temperatures. If the cooling system of the internal combustion engine is of pressure-proof design, such additives may, however, be dispensed with, the heat being carried off as steam at 120° to 165° C. and at a pressure of 2 to 7 atmospheres gage.

Thus a further advantage is offered by the method according to this invention in that, by rising the temperature 20 of the coolant, a heat transfer medium is obtained whose temperature and heat content are sufficient to melt the sulfur which is to be burnt in the internal combustion engine as well as to maintain at an elevated temperature of preferably 145° to 155° C. the apparatus which is 25 required for supplying, purifying and proportioning the molten sulfur.

What we claim is:

1. In the lubrication of moving parts of internal combustion engines operating on sulfur and a gas selected 30 from the group consisting of O<sub>2</sub> and O<sub>2</sub>-containing gases, a method of inhibiting the formation of viscous substances and the corrosion of the moving parts which comprises using a lubricating oil which contains from 0.05 to 10% by weight of sulfur and maintaining the inner 35 surface of the cylinder of the internal combustion engine at a temperature above the dew point of sulfuric acid and below 165° C. by means of a coolant.

2. A method as claimed in claim 1, wherein the coolant used is water to which has been added an agent for elevating the boiling point selected from the group consisting 40 of glycol, glycerol and dimethyl sulfoxide.

3. A method as claimed in claim 1, wherein the coolant used is water which is maintained at a temperature of 120° to 165° C., preferably 145° to 155° C., by the application of pressure.

### References Cited in the file of this patent

#### UNITED STATES PATENTS

|    |           |           |       |               |
|----|-----------|-----------|-------|---------------|
| 50 | 2,222,431 | Colin     | ----- | Nov. 19, 1940 |
|    | 2,231,939 | Nallinger | ----- | Feb. 18, 1941 |
|    | 2,581,050 | Smedslund | ----- | Jan. 1, 1952  |
|    | 2,767,693 | Foutz     | ----- | Oct. 23, 1956 |

#### FOREIGN PATENTS

|    |         |               |       |               |
|----|---------|---------------|-------|---------------|
| 55 | 455,790 | Great Britain | ----- | Oct. 28, 1936 |
|----|---------|---------------|-------|---------------|